

[54] SILVER HALIDE COLOR PHOTOGRAPHIC LIGHT-SENSITIVE MATERIAL

[75] Inventors: Tsumoru Hirano; Makoto Umemoto; Morio Yagihara, all of Kanagawa, Japan

[73] Assignee: Fuji Photo Film Co., Ltd., Kanagawa, Japan

[21] Appl. No.: 501,725

[22] Filed: Jun. 6, 1983

[30] Foreign Application Priority Data

Jun. 4, 1982 [JP] Japan ..... 57-95797

[51] Int. Cl.<sup>3</sup> ..... G03C 7/16; G03C 7/26

[52] U.S. Cl. ..... 430/381; 430/384;

430/385; 430/548; 430/552; 430/553; 430/505

[58] Field of Search ..... 430/381, 384, 385, 548, 430/552, 553, 505

[56] References Cited

U.S. PATENT DOCUMENTS

- |           |         |                      |       |         |
|-----------|---------|----------------------|-------|---------|
| 3,211,552 | 10/1965 | Chu et al.           | ..... | 430/548 |
| 3,370,952 | 2/1968  | Dawson               | ..... | 430/548 |
| 3,451,820 | 6/1969  | Umberger             | ..... | 430/449 |
| 3,767,412 | 10/1973 | Monbalu et al.       | ..... | 430/548 |
| 3,926,436 | 12/1975 | Monbalu et al.       | ..... | 430/548 |
| 4,080,211 | 3/1978  | Van Paesschen et al. | ..... | 430/548 |

Primary Examiner—J. Travis Brown  
Attorney, Agent, or Firm—Sughrue, Mion, Zinn,  
Macpeak & Seas

[57] ABSTRACT

A silver halide color, photographic light-sensitive material comprising a support having thereon a silver halide emulsion layer containing a cyan color image forming polymer coupler latex which is capable of forming a

dye upon coupling with an oxidation product of an aromatic primary amine developing agent and which is a polymer or copolymer having a repeating unit derived from a monomer represented by the following general formula (I):



wherein R<sub>1</sub> represents a hydrogen atom, a lower alkyl group containing from 1 to 4 carbon atoms or a chlorine atom; R<sub>2</sub> represents a hydrogen atom or an unsubstituted or substituted alkyl group having from 1 to 4 carbon atoms; A<sub>1</sub> represents an unsubstituted or substituted alkylene group which may be a straight chain or a branched chain; A<sub>2</sub> represents an unsubstituted or substituted alkylene group which may be a straight chain or a branched chain, an unsubstituted or substituted aralkylene group or an unsubstituted or substituted phenylene group; B<sub>1</sub> represents —O—, —S—, —SO—, —SO<sub>2</sub>—, —CONH— or —COO—; B<sub>2</sub> represents —NHCO— or —OCO—; X represents a halogen atom; Y represents a hydrogen atom or a lower alkyl group having from 1 to 5 carbon atoms; Z represents a hydrogen atom, a halogen atom or a substituted alkoxy group; l represents 0 or 1; m represents 0 or 1; and n represents 0 or 1.

19 Claims, No Drawings

SILVER HALIDE COLOR PHOTOGRAPHIC  
LIGHT-SENSITIVE MATERIAL

## FIELD OF THE INVENTION

The present invention relates to a silver halide color photographic light-sensitive material containing a novel cyan color image forming polymer coupler latex capable of coupling with an oxidation product of an aromatic primary amine developing agent.

## BACKGROUND OF THE INVENTION

It is well known that upon the color development of a silver halide photographic light-sensitive material, after exposure, an oxidized aromatic primary amine developing agent can be reacted with a dye forming coupler to obtain a color image.

It is also known that, for the color development of a silver halide color photographic material, an oxidized aromatic primary amine color developing agent can be reacted with a coupler to form a dye such as an indo-phenol, an indoaniline, an indamine, an azomethine, a phenoxazine, a phenazine, and the like, thus forming a color image. In this procedure, the subtractive color process is ordinarily used for color reproduction, and silver halide emulsions which are selectively sensitive to blue, green and red light, and yellow, magenta and cyan color image formers, which are respectively the complementary colors of blue, green and red, are employed. For example, a coupler of the acylacetanilide or benzoylmethane type is used for forming a yellow color image; a coupler of the pyrazolone, pyrazolobenzimidazole, cyanoacetophenone or indazolone type is generally used for forming a magenta color image; and a phenolic coupler, such as a phenol and a naphthol, is generally used for forming a cyan color image.

Color couplers must satisfy various requirements. For example, it is necessary that they have a good spectral property and provide a dye image having excellent stability to light, temperature, and humidity for a long period of time upon color development.

It is also required in a multilayer color photographic light-sensitive material that each coupler is fixed in a layer separated from each other in order to reduce color mixing and improve color reproduction. Many methods for rendering a coupler diffusion-resistant are known. One method is to introduce a long chain aliphatic group into a coupler molecule in order to prevent diffusion. Couplers according to such a method require a step of addition to an aqueous gelatin solution by solubilizing in alkali, or a step of dispersing in an aqueous gelatin solution by dissolving in a high boiling organic solvent, since the couplers are immiscible with an aqueous gelatin solution. Such color couplers may cause crystal formation in a photographic emulsion. Furthermore, when using a high boiling organic solvent, a large amount of gelatin must be employed since the high boiling organic solvent makes an emulsion layer soft. Consequently, this increases the thickness of the material even though it is desirable to reduce the thickness of the emulsion layer.

Another method for rendering a coupler diffusion-resistant is to utilize a polymer coupler latex obtained by polymerization of a monomeric coupler. An example of a method of adding a polymer coupler in a latex form to a hydrophilic colloid composition is a method in which a latex prepared by an emulsion polymerization method is directly added to a gelatino silver halide emulsion and

a method in which an oleophilic polymer coupler obtained by polymerization of a monomeric coupler is dispersed in a latex form in an aqueous gelatin solution. Some examples of the former emulsion polymerization methods include an emulsion polymerization method in an aqueous gelatin phase as described in U.S. Pat. No. 3,370,952 and an emulsion polymerization method in water as described in U.S. Pat. No. 4,080,211. An example of the latter method in which an oleophilic polymer coupler is dispersed in a latex form is described in U.S. Pat. No. 3,451,820. The method of adding a polymer coupler in a latex form to a hydrophilic colloid composition has many advantages in comparison with other methods. For example, the deterioration of strength of the film formed is small, because the hydrophobic substance is in a latex form. Also, since the latex can contain coupler monomers in a high concentration, it is easy to incorporate couplers in a high concentration into a photographic emulsion, and the increase of viscosity is small. Furthermore, color mixing is prevented, since a polymer coupler is completely immobilized and the crystallization of couplers in the emulsion layer is small.

With respect to the addition of these polymer couplers in a latex form to a gelatino silver halide emulsion, there are described, for example, 4-equivalent magenta polymer coupler latexes and methods of preparation thereof in U.S. Pat. No. 4,080,211, British Pat. No. 1,247,688, and U.S. Pat. No. 3,451,820, copolymer latexes with a competing coupler in West German Pat. No. 2,725,591, and U.S. Pat. No. 3,926,436 and cyan polymer coupler latexes in U.S. Pat. No. 3,767,412 and *Research Disclosure*, No. 21728 (1982). Among these polymer latexes, cyan polymer coupler latexes which are excellent with respect to heat fastness are described in *Research Disclosure*, No. 21728.

However, these cyan polymer coupler latexes have problems to be dissolved as well as many excellent features in addition to the advantages described above, and thus it has been desired to overcome these problems. The problems include the following:

1. The rate of the coupling reaction is poor, and thus sensitivity, gamma and color density of the dye image formed are low.
2. The color reproducibility is inferior because the absorption curve of the cyan dye formed shifts to shorter wavelength side (for example, blue becomes yellowish).

## SUMMARY OF THE INVENTION

Therefore, an object of the present invention is to provide a novel cyan color image forming polymer coupler latex which has an excellent color forming property.

Another object of the present invention is to provide a novel cyan color image forming polymer coupler latex which provides an excellent color reproducibility.

Still another object of the present invention is to provide a color photographic light-sensitive material that forms a color image fast to heat, and heat, and humidity in a color photograph after development processing.

A further object of the present invention is to provide a color photographic light-sensitive material having good film strength.

A further object of the present invention is to provide a color photographic light-sensitive material having a reduced layer thickness and an improved sharpness.

A still further object of the present invention is to provide a method of forming a cyan color image by development of a silver halide emulsion in the presence of a novel cyan dye forming polymer coupler latex.

A still further object of the present invention is to provide a silver halide color photographic light-sensitive material containing a novel cyan dye forming polymer coupler latex, a photographic processing method or an image forming method for using the material.

Other objects of the present invention will be apparent from the following detailed description and examples.

As a result of extensive investigations, it has now been found that these objects of the present invention are accomplished by the use of a cyan color image forming polymer coupler latex which is a polymer or copolymer having a repeating unit derived from a monomer represented by the following general formula (I):



wherein R<sub>1</sub> represents a hydrogen atom, a lower alkyl group containing from 1 to 4 carbon atoms or a chlorine atom; R<sub>2</sub> represents a hydrogen atom or an unsubstituted or substituted alkyl group having from 1 to 4 carbon atoms; A<sub>1</sub> represents an unsubstituted or substituted alkylene group which may be a straight chain or a branched chain; A<sub>2</sub> represents an unsubstituted or substituted alkylene group which may be a straight chain or a branched chain, an unsubstituted or substituted aralkylene group or an unsubstituted or substituted phenylene group; B<sub>1</sub> represents -O-, -S-, -SO-, -SO<sub>2</sub>-, -CONH- or -COO-; B<sub>2</sub> represents -NHCO- or -OCO-; X represents a halogen atom; Y represents a hydrogen atom or a lower alkyl group having from 1 to 5 carbon atoms; Z represents a hydrogen atom, a halogen atom or a substituted alkoxy group; l represents 0 or 1; m represents 0 or 1; and n represents 0 or 1.

In more detail, the objects of the invention can be accomplished with a color photographic light-sensitive material comprising a support having thereon at least one silver halide emulsion layer containing a cyan color image forming polymer coupler latex which is a novel polymer having a repeating unit represented by the general formula (II) described below, or a novel copolymer of the repeating unit described below and a non-color forming unit which does not couple with the oxidation product of an aromatic primary amine developing agent.



wherein R<sub>1</sub>, R<sub>2</sub>, A<sub>1</sub>, A<sub>2</sub>, B<sub>1</sub>, B<sub>2</sub>, X, Y, Z, l, m and n have the same meanings as defined in the general formula (I) above.

#### DETAILED DESCRIPTION OF THE INVENTION

The novel cyan color image forming polymer coupler latex according to the present invention includes a polymer having a repeating unit derived from a monomer coupler represented by the general formula (I), and a copolymer of the repeating unit according to formula (II) and at least one non-color forming unit containing at least one ethylene group which does not have an ability of oxidative coupling with an aromatic primary amine developing agent. Two or more kinds of the monomer couplers can be polymerized together.

In the above-described formula (I), R<sub>1</sub> represents a hydrogen atom, a lower alkyl group having from 1 to 4 carbon atoms, or a chlorine atom; R<sub>2</sub> represents a hydrogen atom or an unsubstituted or substituted alkyl group having from 1 to 4 carbon atoms; A<sub>1</sub> represents an unsubstituted or substituted alkylene group, preferably having from 1 to 10 carbon atoms, which may be a straight chain or a branched chain; A<sub>2</sub> represents an unsubstituted or substituted alkylene group, preferably having from 1 to 10 carbon atoms, which may be a straight chain or a branched chain, an unsubstituted or substituted aralkylene group or an unsubstituted or substituted phenylene group. Examples of the alkylene group for A<sub>1</sub> and A<sub>2</sub> include a methylene group, a methylmethylen group, a dimethylmethylen group, a dimethylen group, a trimethylen group, a tetramethylen group, a pentamethylen group, a hexamethylen group, a decylmethylen group, etc. Example of the aralkylene group for A<sub>2</sub> includes a benzylidene group, etc. Examples of the phenylene group for R<sub>3</sub> include a p-phenylene group, an m-phenylene group, a methylenophenylene group, etc.

B<sub>1</sub> represents -O-, -S-, -SO-, -SO<sub>2</sub>-, -CONH- or -COO-; and B<sub>2</sub> represents -NHCO- or -OCO-.

X represents a halogen atom (for example, a fluorine atom, a chlorine atom, etc.); Y represents a hydrogen atom or a lower alkyl group having from 1 to 5 carbon atoms (for example, a methyl group, an ethyl group, a tert-butyl group, etc.); and Z represents a hydrogen atom, a halogen atom (for example, a fluorine atom, a chlorine atom, etc.) or a substituted alkoxy group. l represents 0 or 1; m represents 0 or 1; and n represents 0 or 1.

Substituents for the alkylene group, the aralkylene group or the phenylene group represented by A<sub>1</sub> or A<sub>2</sub> include an aryl group (for example, a phenyl group, etc.), a nitro group, hydroxy group, a cyano group, a sulfo group, an alkoxy group (for example, a methoxy group, etc.), an aryloxy group (for example, a phenoxy group, etc.), an acyloxy group (for example, an acetoxy

group, etc.), an acylamino group (for example, an acetylaminogroup, etc.), a sulfonamido group (for example, a methanesulfonamido group, etc.), a sulfamoyl group (for example, a methylsulfamoyl group, etc.), a halogen atom (for example, a fluorine atom, a chlorine atom, a bromine atom, etc.), a carboxy group, a carbamoyl group (for example, a methylcarbamoyl group, etc.), an alkoxy carbonyl group (for example, a methoxycarbonyl group, etc.), a sulfonyl group, etc.), a sulfonyl group (for example a methylsulfonyl group, etc.), and the like. When two or more substituents are present, they may be the same or different.

Substituents for the substituted alkoxy group represented by Z include an aryl group (for example, a phenyl group, etc.), a nitro group, a hydroxy group, a cyano group, a sulfo group, an alkoxy group (for example, a methoxy group, etc.), an aryloxy group (for example, a phenoxy group, etc.), an acyloxy group (for example, an acetoxy group, etc.), an acylamino group (for example, an acetylaminogroup, etc.), an alkylsulfonamido group (for example, a methanesulfonamido group, etc.), an alkylsulfamoyl group (for example, a methylsulfamoyl group, etc.), a halogen atom (for example, a fluorine atom, a chlorine atom, a bromine atom, etc.), a carboxy group, an alkylcarbamoyl group (for example, a methylcarbamoyl group, etc.), an alkoxycarbonyl group (for example, a methoxycarbonyl group, etc.), an alkylsulfonyl group (for example, a methylsulfonyl group, etc.), an alkylthio group (for example, an ethylthio group, etc.), and the like. When two or more substituents are present, they may be the same or different.

Of the monomer couplers represented by the general formula (I), those represented by the general formula (I') described below are particularly preferred.



wherein R<sub>1</sub>, R<sub>2</sub>, A<sub>1</sub>, X, Y and Z have the same meanings as defined above.

Examples of the non-color forming ethylenic monomer which does not couple with the oxidation product of an aromatic primary amine developing agent include an ester and an amide, derived from an acrylic acid, for example, acrylic acid, an  $\alpha$ -chloroacrylic acid, an  $\alpha$ -alkylacrylic acid such as methacrylic acid, etc. (for example, acrylamide, methacrylamide, n-butylacrylamide, t-butylacrylamide, diacetoneacrylamide, methyl acrylate, ethyl acrylate, n-propyl acrylate, n-butyl acrylate, t-butyl acrylate, isobutyl acrylate, 2-ethylhexyl acrylate, n-octyl acrylate, lauryl acrylate, methyl methacrylate, ethyl methacrylate, n-butyl methacrylate,  $\beta$ -hydroxymethacrylate, etc.), a vinyl ester (for example, vinyl acetate, vinyl propionate, vinyl laurate, etc.), acrylonitrile, methacrylonitrile, an aromatic vinyl compound (for example, styrene and a derivative thereof, for example, vinyl toluene, divinyl benzene, vinyl acetophenone, sulfostyrene, etc.), itaconic acid, citraconic acid, crotonic acid, vinylidene chloride, a vinyl alkyl ether (for example, vinyl ethyl ether, etc. an ester of maleic acid, N-vinyl-2-pyrrolidone, N-vinylpyridine, 2- or 4-vinylpyridine, etc.

Of these monomers, an ester of acrylic acid, an ester of methacrylic acid, an ester of maleic acid are particularly preferred.

Two or more non-color forming ethylenically unsaturated monomers described above can be used together. For example, a combination of methyl acrylate and diacetoneacrylamide, methyl acrylate and methacrylic acid, styrene and n-butyl acrylate, etc., can be employed.

The ethylenically unsaturated monomer which is used to copolymerize with the monomer coupler represented by the above-described general formula (I) can be selected so that the copolymer to be formed possesses good physical properties and/or chemical properties, for example, solubility, compatibility with a binder such as gelatin in a photographic colloid composition, flexibility, heat stability, etc., as well known in the field of polymer color couplers.

The cyan polymer coupler latex used in the present invention can be prepared by dissolving an oleophilic polymer coupler obtained by polymerization of a monomer coupler in an organic solvent and then dispersing the solution in a latex form in an aqueous gelatin solution, or can be directly prepared by an emulsion polymerization method. With respect to the method in which an oleophilic polymer coupler is dispersed in a latex form in an aqueous gelatin solution, the method as described in U.S. Pat. No. 3,451,820 and with respect to the emulsion polymerization, the methods as described in U.S. Pat. Nos. 4,080,211 and 3,370,952 can be employed, respectively. These methods can be applied to preparation of homopolymers and preparation of copolymers. In the latter case, a non-color forming monomer is preferably a liquid monomer which may act, in the case of the emulsion polymerization, as a solvent for a monomer which is normally solid.

Free radical polymerization of an ethylenically unsaturated solid monomer is initiated with the addition to the monomer molecule of a free radical which is formed by thermal decomposition of a chemical initiator, an action of a reducing agent to an oxidative compound (a redox initiator) or a physical action, for example, irradiation of ultraviolet rays or other high energy radiations, high frequencies, etc.

Examples of the chemical initiators commonly used include a water-soluble initiator, for example, a persulfate (such as ammonium persulfate, potassium persulfate, etc.), hydrogen peroxide, 4,4'-azobis(4-cyanovaleric acid), etc., and a water-insoluble initiator, for example, azobisisobutyronitrile (such as 2,2'-azobis(2,4-dimethylvaleronitrile), 2,2'-azobisisobutyronitrile, etc.), benzoyl peroxide, chlorobenzoyl peroxide, and other compounds. Examples of the redox initiators usually used include hydrogen peroxide-iron (II) salt, potassium persulfate-potassium hydrogensulfate, cerium salt-alcohol, etc. Specific examples and functions of the initiators are described in F. A. Bovey, *Emulsion Polymerization*, pages 59-93, (Interscience Publishers Inc., New York (1955)).

Organic solvents which can be used in polymerization of the oleophilic cyan polymer couplers are preferably those which can usually be admixed with monomers to be used without limitation, are good solvent for the oleophilic polymer coupler formed, do not react with initiators to be used and do not interrupt usual actions in free radical addition polymerization.

Specific examples of the organic solvent which can be used include an aromatic hydrocarbon (for example,

benzene, toluene, etc.), a hydrocarbon (for example, n-hexane, etc.), an alcohol (for example, methanol, ethanol, isopropanol, tert-butanol, etc.), a ketone (for example, acetone, methyl ethyl ketone, etc.), a cyclic ether (for example, tetrahydrofuran, dioxan, etc.), an ester (for example, ethyl acetate, etc.), a chlorinated hydrocarbon (for example, methylene chloride, chloroform, etc.), an amide (for example, dimethylformamide, dimethylacetamide, etc.), a sulfoxide (for example, dimethylsulfoxide, etc.), a nitrile (for example, acetonitrile, etc.), and a mixture thereof.

On the other hand, emulsion polymerization of solid water-insoluble monomer couplers is usually carried out in an aqueous system or a water/organic solvent system. Organic solvents which can be used are preferably those which are substantially inert to solid water-insoluble monomer couplers to be used, do not interrupt usual actions in free radical addition polymerization and have a low boiling point so as to be capable of being easily removed from an aqueous reaction medium by distillation during and/or after polymerization. Preferred examples include a lower alcohol having from 1 to 4 carbon atoms (for example, methanol, ethanol, isopropanol, etc.), a ketone (for example, acetone, etc.), a chlorinated hydrocarbon (for example, chloroform, etc.), an aromatic hydrocarbon (for example, benzene, etc.), a cyclic ether (for example, tetrahydrofuran, etc.), an ester (for example, ethyl acetate, etc.), a nitrile (for example, acetonitrile, etc.), and the like.

Further, an organic solvent which is used for dissolving an oleophilic polymer coupler in the case where the oleophilic polymer coupler is dispersed in a latex form in an aqueous gelatin solution is removed from the mixture before coating of the dispersion solution or by vaporization during drying of the dispersion solution coated, although the latter is less preferable. With respect to removing the solvent, a method in which the solvent is removed by washing a gelatin noodle with water is applied when the solvent is water-soluble to some extent, or a spray drying method, a vacuum purging method or a steam purging method can be employed for removing the solvent.

Examples of the organic solvents which can be removed include, for example, an ester (for example, a lower alkyl ester, etc.), a lower alkyl ether, a ketone, a halogenated hydrocarbon (for example, methylene chloride, trichloroethylene, a fluorinated hydrocarbon, etc.), an alcohol (for example, an alcohol between n-butyl alcohol and octyl alcohol, etc.), and a mixture thereof.

50

Any type of dispersing agent can be used in the dispersion of the oleophilic polymer coupler, Ionic surface active agents, and particularly anionic surface active agents are preferred. Amphoteric surface active agents such as C-cetyl betaine, an N-alkylaminopropionate, an N-alkyliminodipropionate, etc., can also be used.

As an emulsifier which can be used in the emulsion polymerization, a compound having surface activity is used. Preferred examples include soap, a sulfonate, a sulfate, a cationic compound, an amphoteric compound and a high molecular weight protective colloid. Specific examples and functions of the emulsifiers are described in *Belgische Chemische Industrie*, Vol. 28, pages 16-20 (1963).

In order to increase the dispersion stability, to improve the color forming property of a polymer coupler latex dispersed, control the color hue of a dye formed from a polymer coupler latex dispersed and the oxida-

tion product of an aromatic primary amine developing agent and improve the bending property of the emulsion coated, a permanent solvent, that is, a water-immiscible organic solvent having a high boiling point (i.e., above 200° C.), may be added in a small amount. The concentration of the permanent solvent must be at such a low level that the copolymer is plasticized while it is maintained in solid particle form. Furthermore, it is desirable to use the permanent solvent in a relatively low concentration in order to reduce the thickness of a final emulsion layer as much as possible to obtain good sharpness.

It is desirable that the ratio of the color forming portion in the polymer coupler latex is usually from 5 to 80% by weight. Particularly, a ratio from 20 to 70% by weight is preferred in view of color reproducibility, color forming property and stability. In this case, an equivalent molecular weight, that is, a gram number of the polymer containing 1 mol of a monomer coupler is preferably from about 250 to 4,000, but it is not limited thereto.

Preferred specific examples of the monomer couplers used in the present invention are set forth below, but the present invention is not to be construed as being limited thereto.



-continued



-continued



5

(8)

(9)

10 The monomer coupler corresponding to the general formula (I) according to the present invention can be synthesized in the following reaction scheme:



10 40 In the above formulae, R<sub>1</sub>, R<sub>2</sub>, A<sub>1</sub>, A<sub>2</sub>, B<sub>1</sub>, B<sub>2</sub>, X, Y, Z, l, m and n each has the same meaning as defined above and X' represents a halogen atom (for example, a chlorine atom, a bromine atom, etc.).

That is, the monomer coupler can be synthesized by reacting a 2-aminophenol derivative represented by the general formula (III) with an acid chloride represented by the general formula (IV), or through an intermediate product represented by the general formula (VII) which is obtained by reacting a 2-aminophenol derivative represented by the general formula (III) with an acid chloride represented by the general formula (IV).

10 45 50 Typical synthesis examples of the monomer compounds and the polymer compounds according to the present invention are set forth below.

#### A. Monomer Compounds

#### 55 SYNTHESIS EXAMPLE 1

##### Synthesis of

##### 6-( $\alpha$ -acrylamidoacetamido)-2,4-dichloro-3-methylphenol [Monomer Coupler (1)]

60 In a mixture composed of 80 g (2.0 mol) and 200 ml of water was dissolved with stirring 165 g (2.2 mol) of glycine and the mixture was cooled to 0° C. To the aqueous solution, there were simultaneously added dropwise 254 g (2.0 mol) of  $\beta$ -chloropropionyl chloride

65 and an aqueous solution containing 127.2 g (1.2 mol) of sodium carbonate dissolved in 400 ml of water. After the completion of the reaction, 1 liter of acetonitrile was added to the reaction solution and the mixture was then



acidified by adding 200 ml of concentrated hydrochloric acid. 1 liter of acetonitrile was further added to extract and the acetonitrile layer was separated. The acetonitrile solution was concentrated and the crystals thus deposited were collected and recrystallized from ethyl acetate to obtain 235.3 g of N-( $\beta$ -chloropropanoyl)glycine.

To a mixture composed of 158 g (0.96 mol) of N-( $\beta$ -chloropropanoyl)glycine thus obtained and 92 g (0.4 mol) of 6-amino-2,4-dichloro-3-methylphenol hydrochloride were added 228 ml (2.88 mol) of pyridine and 2 liters of acetonitrile and stirred under cooling. To the solution was added dropwise 95.2 g (0.8 mol) of thionyl chloride. After the completion of the reaction, water was added to the reaction solution and the crystals thus deposited were collected by filtration and recrystallized from acetonitrile to obtain 125.2 g of 6-[ $\alpha$ -( $\beta$ -chloropropanamido)acetamido]-2,4-dichloro-3-methylphenol.

35.6 g (0.64 mol) of potassium hydroxide was dissolved in 1.3 liters of methanol and the solution was cooled with ice with stirring to which was added 43.2 g (0.127 mol) of the  $\beta$ -chloropropanamido compound obtained in the above described manner. After stirring for about 30 minutes, the mixture was neutralized with acetic acid and to which was added 1 liter of water. The crystals thus deposited were collected by filtration and recrystallized from a solvent mixture of ethanol and ethyl acetate to obtain 28.0 g of Monomer Coupler (1).

Melting Point: 225° to 227° C.

Elemental Analysis for C<sub>12</sub>H<sub>12</sub>Cl<sub>2</sub>N<sub>2</sub>O<sub>3</sub>: Calculated: C: 47.54%, H: 3.99%, N: 9.25%. Found: C: 47.73%, H: 4.02%, N: 9.16%.

## SYNTHESIS EXAMPLE 2

### Synthesis of

#### 6-( $\alpha$ -methacrylamidoacetamido)-2,4-dichloro-3-methylphenol [Monomer Coupler 2]

In a mixture composed of 80 g (2.0 mol) of sodium hydroxide, 400 ml of water and 4 ml of nitrobenzene was dissolved with stirring 150 g (2.0 mol) of glycine and the mixture was cooled to 0° C. To the aqueous solution, there were simultaneously added dropwise 230 g (2.2 mol) of methacrylic chloride and an aqueous solution containing 96 g (2.4 mol) of sodium hydroxide dissolved in 200 ml of water. After the completion of the reaction, 800 ml of acetonitrile was added to the reaction solution and the mixture was then acidified by adding 160 ml of concentrated hydrochloric acid. 1 liter of acetonitrile was further added to extract and the acetonitrile layer was separated. The acetonitrile solution was concentrated and the crystals thus deposited were collected and recrystallized from ethyl acetate to obtain 117 g of N-methacryloyl glycine.

To mixture composed of 68 g (0.48 mol) of N-methacryloyl glycine obtained in the above described manner and 46 g (0.2 mol) of 6-amino-2,4-dichloro-3-methylphenol hydrochloride were added 114 ml (1.44 mol) of pyridine and 1 liter of ethyl acetate and stirred under cooling. To the solution was added dropwise 29 ml (0.4 mol) of thionyl chloride. After the completion of the reaction, 300 ml of water was added to the reaction solution and extracted with ethyl acetate. The ethyl acetate solution was concentrated and to the residue was added acetonitrile. The crystals thus deposited were collected and recrystallized from acetonitrile to obtain 34.8 g of Monomer Coupler (2).

Melting Point: 217° to 218° C.

Elemental Analysis for C<sub>13</sub>H<sub>14</sub>Cl<sub>2</sub>N<sub>2</sub>O<sub>3</sub>: Calculated: C: 49.23%, H: 4.45%, N: 8.83%. Found: C: 49.18%, H: 4.43%, N: 8.95%.

## SYNTHESIS EXAMPLE 3

### Synthesis of

#### 6-(2-methacrylamidopropanamido)-2,4-dichloro-3-methylphenol [Monomer Coupler (3)]

10 N-methacryloyl- $\alpha$ -alanine was obtained in the same manner as described in Synthesis Example 2 but using alanine as a starting material.

15 To a mixture composed of 76 g (0.48 mol) of N-methacryloyl- $\alpha$ -alanine obtained above and 46 g (0.2 mol) of 6-amino-2,4-dichloro-3-methylphenol hydrochloride were added 114 ml (1.44 mol) of pyridine and 1 liter of ethyl acetate and stirred under cooling. To the solution was added dropwise 29 ml (0.4 mol) of thionyl chloride. After the completion of the reaction, 300 ml of water was added to the reaction solution and extracted with ethyl acetate. The ethyl acetate solution was concentrated and the crystals thus deposited were collected and recrystallized from a solvent mixture of ethyl acetate and ethanol to obtain 40.1 g of Monomer Coupler (3).

20 Melting Point: 190° to 193° C.

Elemental Analysis for C<sub>14</sub>H<sub>16</sub>Cl<sub>2</sub>N<sub>2</sub>O<sub>3</sub>: Calculated: C: 50.77%, H: 4.84%, N: 8.46%. Found: C: 51.04%, H: 4.96%, N: 8.37%.

## SYNTHESIS EXAMPLE 4

### Synthesis of

#### 6-(4-methacrylamidobutanamido)-2,4-dichloro-3-methylphenol Monomer Coupler (8)

35 In a mixture composed of 80 g (2.0 mol) of sodium hydroxide, 400 ml of water and 4 ml of nitrobenzene was dissolved with stirring 214 g (2.0 mol) of  $\gamma$ -aminobutyric acid and the mixture was cooled to 0° C. To the aqueous solution, there were simultaneously added dropwise 230 g (2.2 mol) of methacrylic chloride and an aqueous solution containing 96 g (2.4 mol) of sodium hydroxide dissolved in 200 ml of water. After the completion of the reaction, 800 ml of acetonitrile was added to the reaction solution and the mixture was then acidified by adding 160 ml of concentrated hydrochloric acid. 1 liter of acetonitrile was further added to extract and the acetonitrile layer was separated. The acetonitrile solution was concentrated to obtain 318.4 g of N-methacryloyl- $\gamma$ -aminobutyric acid as an oily product.

40 In the same manner as described in Synthesis Example 2 but using 82 g (0.48 mol) of N-methacryloyl- $\gamma$ -aminobutyric acid obtained in the above described manner, 49.3 g of Monomer Coupler (8) was obtained.

Melting Point: 119° to 121° C.

45 Elemental Analysis for C<sub>15</sub>H<sub>18</sub>Cl<sub>2</sub>N<sub>2</sub>O<sub>3</sub>: Calculated: C: 52.18%, H: 5.25%, N: 8.12%. Found: C: 52.14%, H: 5.72%, N: 8.14%.

## SYNTHESIS EXAMPLE 5

### Synthesis of

#### 6-(6-methacrylamidohexanamido)-2,4-dichloro-3-methylphenol [Monomer Coupler (9)]

50  $\epsilon$ -Methacryloylaminocaproic acid was obtained as an oily product in the same manner as described in Synthesis Example 3 but using  $\epsilon$ -aminocaproic acid as a starting material.

To a mixture composed of 192 g (0.96 mol) of  $\epsilon$ -methacryloylaminocaproic acid obtained above and 92 g (0.4 mol) of 6-amino-2,4-dichloro-3-methylphenol hydrochloride were added 228 ml (2.88 mol) of pyridine and 2 liters of ethyl acetate and stirred under cooling. To the solution was added dropwise 58 ml (0.8 mol) of thionyl chloride. After the completion of the reaction, 2 liters of water was added to the reaction solution and extracted with ethyl acetate. The ethyl acetate solution was concentrated, to the residue was added 1 liter of methanol and the mixture was stirred under cooling. To the solution was added 300 ml of a methanol solution containing 26 g of potassium hydroxide dissolved and the mixture was stirred for about 30 minutes and neutralized with acetic acid. 1.6 liters of water was added to the mixture and the crystals thus deposited were collected and recrystallized from ethyl acetate to obtain 106.5 g of Monomer Coupler (9).

Melting Point: 111° to 115° C.

Elemental Analysis for  $C_{17}H_{22}Cl_2N_2O_3$ : Calculated: C: 54.70%, H: 5.94%, N: 7.51%. Found: C: 54.87%, H: 5.99%, N: 7.48%.

#### B. Polymer Compounds

##### Synthesis Method I

##### SYNTHESIS EXAMPLE 6

###### Synthesis of copolymer coupler of

6-( $\alpha$ -methacrylamidoacetamido)-2,4-dichloro-3-methylphenol [Monomer Coupler (2)], methyl acrylate 30 and diacetoneacrylamide [Oleophilic Polymer Coupler (A)]

A mixture composed of 20 g of Monomer Coupler (2), 16 g of methyl acrylate, 4 g of diacetoneacrylamide and 200 ml of dioxane was heated to 80° C. with stirring while introducing nitrogen gas. To the mixture was added 10 ml of a dioxane containing 300 mg of azobisisobutyronitrile dissolved to initiate polymerization. After reacting for 5 hours, the reaction solution was 40 cooled and poured into 2 liters of water. The solid thus deposited were collected by filtration and thoroughly washed with water. By drying the solid under a reduced pressure with heating, 37.7 g of Oleophilic Polymer Coupler (A) was obtained. It was found that the oleophilic polymer coupler contained 52.3% of Monomer Coupler (2) in the copolymer synthesized as the result of chlorine analysis.

A method for dispersing Oleophilic Polymer Coupler (A) in an aqueous gelatin solution in a form of latex is 50 described in the following.

###### Synthesis of Polymer Coupler Latex (A')

Two solutions (a) and (b) were prepared in the following manner.

Solution (a): 300 g of a 5% by weight aqueous solution of bone gelatin (pH of 5.6 at 35° C.) was heated to 32° C. and to which was added 12 ml of a 10% by weight aqueous solution of sodium lauryl sulfate.

Solution (b): 20 g of Oleophilic Polymer Coupler (A) described above was dissolved in 60 g of ethyl acetate at 38° C.

Solution (b) was put into a mixer with explosion preventing equipment while stirring at a high speed to which was rapidly added solution (a). After stirring for 1 minute, the mixer was stopped and ethyl acetate was removed by distillation under a reduced pressure. Thus, the oleophilic polymer coupler was dispersed in a di-

luted gelatin solution to prepare Polymer Coupler Latex (A').

##### SYNTHESIS EXAMPLE 7

Synthesis of copolymer coupler of 6-( $\alpha$ -methacrylamidoacetamido)-2,4-dichloro-3-methylphenol [Monomer Coupler (8)] and methyl acrylate [Oleophilic Polymer Coupler (B)]

A mixture composed of 30 g of Monomer Coupler (8), 30 g of methyl acrylate and 300 g of dioxane was heated to 80° C. with stirring while introducing nitrogen gas. To the mixture was added 10 ml of dioxane containing 600 mg of azobisisobutyronitrile dissolved to initiate polymerization. After reacting for 3 hours the temperature was raised to 100° C. and the mixture was further reacted for 2 hours. The reaction solution was cooled and poured into 2 liters of water. The solid thus deposited was collected by filtration and thoroughly washed with water. By drying the solid under a reduced pressure with heating, 56.8 g of Oleophilic Polymer Coupler (B) was obtained. It was found that the oleophilic polymer coupler contained 52.9% of Monomer Coupler (8) in the copolymer synthesized as the result of chlorine analysis.

A method for dispersing Oleophilic Polymer Coupler (B) in an aqueous gelatin solution in a form of latex is described in the following.

###### Synthesis of Polymer Coupler Latex (B')

Two solutions (a) and (b) were prepared in the following manner.

Solution (a): 200 g of a 3.0% by weight aqueous solution of bone gelatin (pH of 5.6 at 35° C.) was heated to 38° C. and to which was added 16 ml of a 10% by weight aqueous solution of sodium lauryl sulfate.

Solution (b): 20 g of Oleophilic Polymer Coupler (B) described above was dissolved in 200 ml of ethyl acetate at 38° C.

Solution (b) was put into a mixer with explosion preventing equipment while stirring at high speed and to which was rapidly added Solution (a). After stirring for 1 minute, the mixer was stopped and ethyl acetate was removed by distillation under a reduced pressure. Thus, the oleophilic polymer coupler was dispersed in a diluted gelatin solution to prepare Polymer Coupler Latex (B').

##### SYNTHESIS EXAMPLE 8

Synthesis of copolymer coupler of 6-( $\alpha$ -methacrylamidoacetamido)-2,4-dichloro-3-methylphenol [Monomer Coupler (8)], methyl acrylate and diacetoneacrylamide [Oleophilic Polymer Coupler (C)]

A mixture composed of 150 g of Monomer Coupler (8), 90 g of methyl acrylate, 60 g of diacetoneacrylamide and 1.5 liters of dioxane was heated to 80° C. with stirring while introducing nitrogen gas. To the mixture was added 50 ml of dioxane containing 3 g of azobisisobutyronitrile dissolved to initiate polymerization. After reacting for 3 hours, the temperature was raised to 100° C. and the mixture was further reacted for 2 hours. The reaction solution was cooled and poured into 10 liters of ice water. The solid thus deposited was collected by filtration and thoroughly washed with water. By drying the solid under a reduced pressure with heating, 281 g of Oleophilic Polymer Coupler (C) was obtained. It was found that the oleophilic polymer coupler contained

50.4% of Monomer Coupler (8) in the copolymer synthesized as the result of chlorine analysis.

A method for dispersing Oleophilic Polymer Coupler (C) in an aqueous gelatin solution in a form of latex is described in the following.

5

#### Synthesis of Polymer Coupler Latex (C')

Two solutions (a) and (b) were prepared in the following manner.

Solution (a): 200 g of a 3.0% by weight aqueous solution of bone gelatin (pH of 5.6 at 35° C.) was heated to 38° C. and to which was added 16 ml of a 10% by weight aqueous solution of sodium lauryl sulfate.

Solution (b): 20 g of Oleophilic Polymer Coupler (C) described above was dissolved in 200 ml of ethyl acetate at 38° C.

Solution (b) was put into a mixer with explosion preventing equipment while stirring at high speed and to which was rapidly added Solution (a). After stirring for 1 minute, the mixer was stopped and ethyl acetate was removed by distillation under a reduced pressure. Thus, the oleophilic polymer coupler was dispersed in a diluted gelatin solution to prepare Polymer Coupler Latex (C').

25

#### SYNTHESIS EXAMPLES 9 TO 25

Using the above-described monomer couplers, the oleophilic cyan polymer couplers described below were prepared in the same manner as described for the copolymers in Synthesis Examples 6, 7 and 8 (Synthesis 30 Method I).

#### SYNTHESIS EXAMPLE 26

Synthesis of copolymer coupler latex of 6-(2-acrylamidoacetamido)-2,4-dichloro-3-methylphenol [Monomer Coupler (1)] and ethyl acrylate [Polymer Coupler Latex (I)]

A solution composed of 30 g of Monomer Coupler (1), 45 g of ethyl acrylate, 3.75 g of oleyl methyl tauride and 750 ml of water was heated to 80° C. with stirring while introducing nitrogen gas in a 1 liter flask. To the mixture was added 23 ml of a 2% aqueous solution of potassium persulfate to initiate polymerization. After reacting for 1 hour, 10 ml of a 2% aqueous solution of potassium persulfate was added. After further reacting for 1 hour, the ethyl acrylate not reacted was distilled off. The latex thus-formed was cooled, pH of which was adjusted to 6.0 with a 1N sodium hydroxide solution and filtered. The concentration of the polymer in the latex formed was 9.8% and it was found that the polymer contained 40.6% of Monomer Coupler (1) as the result of chlorine analysis.

#### SYNTHESIS EXAMPLE 27

Synthesis of copolymer coupler latex of 6-(4-methacrylamidobutanamido)-2,4-dichloro-3-methylphenol [Monomer Coupler (8)] and methyl acrylate [Polymer Coupler Latex (II)]

400 ml of an aqueous solution containing 2.2 g of oleyl methyl tauride dissolved was heated to 80° C. with stirring while introducing nitrogen gas in a 1 liter flask.

| Oleophilic Polymer Coupler by Synthesis Method I |                            |                 |            |               |            |                                        |
|--------------------------------------------------|----------------------------|-----------------|------------|---------------|------------|----------------------------------------|
| Synthesis Example                                | Oleophilic Polymer Coupler | Monomer Coupler | Amount (g) | (*) Comonomer | Amount (g) | Monomer Coupler Unit in Polymer (wt %) |
| 9                                                | D                          | (1)             | 20         | MMA           | 25         | 42.4                                   |
|                                                  |                            |                 |            | MAA           | 5          |                                        |
| 10                                               | E                          | (2)             | 20         | MA            | 16         | 50.8                                   |
|                                                  |                            |                 |            | DAAM          | 4          |                                        |
| 11                                               | F                          | (2)             | 20         | MA            | 20         | 51.9                                   |
| 12                                               | G                          | (3)             | 20         | n-BAM         | 80         | 22.6                                   |
| 13                                               | H                          | (3)             | 20         | MA            | 20         | 52.5                                   |
| 14                                               | I                          | (4)             | 20         | BA            | 20         | 52.3                                   |
| 15                                               | J                          | (5)             | 20         | MA            | 20         | 51.7                                   |
| 16                                               | K                          | (6)             | 20         | EHA           | 10         | 52.8                                   |
|                                                  |                            |                 |            | t-BAM         | 10         |                                        |
| 17                                               | L                          | (7)             | 20         | IBA           | 30         | 41.3                                   |
| 18                                               | M                          | (8)             | 20         | MA            | 16         | 50.9                                   |
|                                                  |                            |                 |            | DAAM          | 4          |                                        |
| 19                                               | N                          | (9)             | 20         | MA            | 20         | 51.3                                   |
| 20                                               | O                          | (10)            | 20         | MMA           | 25         | 43.1                                   |
|                                                  |                            |                 |            | AA            | 5          |                                        |
| 21                                               | P                          | (11)            | 20         | BA            | 15         | 60.2                                   |
| 22                                               | Q                          | (12)            | 20         | EHA           | 30         | 40.5                                   |
| 23                                               | R                          | (13)            | 20         | MA            | 30         | 42.2                                   |
| 24                                               | S                          | (14)            | 20         | EMA           | 20         | 50.9                                   |
| 25                                               | T                          | (15)            | 20         | MA            | 20         | 51.8                                   |

The amounts of the monomer couplers and the comonomers in the above table indicate amounts used in the synthesis of the oleophilic polymer couplers.

Dispersion of these oleophilic polymer couplers in 65 latexes can be carried out in the same manner as described in Synthesis Examples 6, 7 and 8.

#### Synthesis Method II

To the aqueous solution were added 2 ml of a 2% aqueous solution of potassium persulfate and 4 g of methyl acrylate. After 1 hour, 20 g of Monomer Coupler (8), 20 g of methyl acrylate and 200 ml of ethanol were added and then 14 ml of a 2% aqueous solution of potassium persulfate was added. After 1 hour, 6 ml of a 2% aqueous solution of potassium persulfate was added. After further reacting for 1 hour, the methyl acrylate not reacted and the ethanol was distilled off. The latex thus-formed was cooled, pH of which was adjusted to 6.0 with a 1N sodium hydroxide solution and filtered.

The concentration of the polymer in the latex formed was 10.7% and it was found that the polymer contained 46.3% of Monomer Coupler (8) as the result of chlorine analysis.

#### SYNTHESIS EXAMPLE 28

Synthesis of copolymer coupler latex of 6-(6-methacrylamido hexanamido)-2,4-dichloro-3-methylphenol Monomer Coupler (9) and t-butyl acrylamide Polymer Coupler Latex (III)

450 ml of an aqueous solution containing 1.5 g of oleyl methyl tauride dissolved was heated to 85°C with stirring while introducing nitrogen gas in a 1 liter flask. To the aqueous solution was added 10 ml of a 2% aqueous solution of potassium persulfate and then was added dropwise over a period of 20 minutes a solution prepared by dissolving with heating 10 g of Monomer Coupler (9) and 15 g of t-butylacrylamide in 150 ml of ethanol. After 1 hour, 4 ml of a 2% aqueous solution of potassium persulfate was added. After further reacting for 1 hour, the ethanol was distilled off. The latex thus formed was cooled, pH of which was adjusted to 6.0 with a 1N sodium hydroxide solution and filtered. The concentration of the polymer in the latex formed was 6.1% and it was found that the polymer contained 40.2% of Monomer Coupler (9) as the result of chlorine analysis.

#### SYNTHESIS EXAMPLES 29 TO 40

Using the above-described monomer couplers, the cyan polymer coupler latexes described below were prepared in the same manner as described for the copolymers in Synthesis Examples 26, 27 and 28 (Synthesis Method II).

The cyan polymer coupler latexes according to the present invention can be used individually or as mixtures of two or more thereof.

- The cyan polymer coupler latexes according to the present invention can also be used together with a cyan polymer coupler latex, such as those described in U.S. Pat. No. 4,080,211, West German Pat. No. 2,725,591, U.S. Pat. No. 3,926,436 and *Research Disclosure*, No. 21728, etc.
- 5 Further, a dispersion which is prepared by dispersing a hydrophobic cyan color forming coupler such as a phenol coupler or a naphthol coupler, for example, a cyan coupler, as described in U.S. Pat. Nos. 2,369,929, 2,434,272, 2,474,293, 2,521,908, 2,895,826, 3,034,892, 15 3,311,476, 3,458,315, 3,476,563, 3,583,971, 3,591,383, 3,767,411 and 4,004,929, West German Patent Application (OLS) Nos. 2,414,830 and 2,454,329, Japanese Patent Application (OPI) Nos. 59838/73, 26034/76, 5055/73, 146828/76 and 73050/80, etc., in a hydrophilic 20 colloid in a manner as described, for example, in U.S. Pat. Nos. 2,269,158, 2,272,191, 2,304,940, 2,311,020, 2,322,027, 2,360,289, 2,772,163, 2,801,170, 2,801,171 and 3,619,195, British Pat. No. 1,151,590, West German Pat. No. 1,143,707, etc., is loaded into the cyan polymer 25 coupler latex according to the present invention in a manner as described in Japanese Patent Application (OPI) No. 39853/76, etc., and the resulting latex can be used. It is also possible for the above-described hydrophobic cyan coupler to be loaded into the cyan polymer 30 coupler latex according to the present invention in a manner as described in Japanese Patent Application (OPI) Nos. 59942/76 and 32552/79, U.S. Pat. No. 4,199,363, etc., and the resulting latex can be used. The term "load" used herein refers to the state in which a

Polymer Coupler Latexes by Synthesis Method II

| Synthesis Example | Polymer Coupler Latex | Monomer Coupler | Amount (g) | *(1) Comonomer | Amount (g) | Monomer Coupler Unit in Polymer (wt %) |
|-------------------|-----------------------|-----------------|------------|----------------|------------|----------------------------------------|
| 29                | (IV)                  | (1)             | 20         | BA             | 30         | 40.2                                   |
| 30                | (V)                   | (2)             | 20         | MA             | 20         | 50.8                                   |
| 31                | (VI)                  | (3)             | 20         | BA             | 25         | 42.6                                   |
|                   |                       |                 |            | MAA            | 5          |                                        |
| 32                | (VII)                 | (6)             | 20         | MA             | 12         | 48.1                                   |
|                   |                       |                 |            | DAAM           | 8          |                                        |
| 33                | (VIII)                | (7)             | 20         | EA             | 30         | 42.3                                   |
| 34                | (IX)                  | (8)             | 20         | MA             | 16         | 44.8                                   |
|                   |                       |                 |            | DAAM           | 4          |                                        |
| 35                | (X)                   | (9)             | 20         | t-BAM          | 40         | 35.6                                   |
| 36                | (XI)                  | (11)            | 20         | EHA            | 30         | 40.1                                   |
| 37                | (XII)                 | (12)            | 20         | BA             | 25         | 41.8                                   |
|                   |                       |                 |            | MAA            | 5          |                                        |
| 38                | (XIII)                | (13)            | 20         | MA             | 20         | 46.5                                   |
| 39                | (XIV)                 | (14)            | 20         | EMA            | 30         | 40.3                                   |
| 40                | (XV)                  | (15)            | 20         | IBA            | 20         | 40.2                                   |

The amounts of the monomer couplers and the comonomers in the above table indicate amounts used in the synthesis of the polymer coupler latexes.

|         |                       |       |                    |
|---------|-----------------------|-------|--------------------|
| *(1) MA | Methyl Acrylate       | EA    | Ethyl Acrylate     |
| BA      | Butyl Acrylate        | IBA   | i-butyl Acrylate   |
| EHA     | 2-Ethylhexyl Acrylate |       |                    |
| MMA     | Methyl Methacrylate   | EMA   | Ethyl Methacrylate |
| n-BAM   | n-Butylacrylamide     | t-BAM | t-Butylacrylamide  |
| DAAM    | Diacetoneacrylamide   | AA    | Acrylic Acid       |
| MAA     | Methacrylic Acid      |       |                    |

hydrophobic cyan coupler is incorporated into the interior of a cyan polymer coupler latex, or a state in which a hydrophobic cyan coupler is deposited on the surface 60 of a cyan polymer coupler latex. However, the mechanism by which the load occurs is not accurately known.

In order to satisfy the characteristics required of the photographic light-sensitive material, a dispersion which is prepared by dispersing a development inhibitor releasing (DIR) coupler as described, for example, in U.S. Pat. Nos. 3,148,062, 3,227,554, 3,733,201, 3,617,291, 3,703,375, 3,615,506, 3,265,506, 3,620,745, 3,632,345, 3,869,291, 3,642,485, 3,770,436 and 3,808,945,

British Pat. Nos. 1,201,110 and 1,236,767, etc., in a hydrophilic colloid in a manner as described in U.S. Pat. Nos. 2,269,158, 2,272,191, 2,304,940, 2,311,020, 2,322,027, 2,360,289, 2,772,163, 2,801,170, 2,801,171 and 3,619,195, British Pat. No. 1,151,590, West German Pat. No. 1,143,707, etc., is loaded into the cyan polymer coupler latex according to the present invention in a manner as described in Japanese Patent Application (OPI) No. 39853/76. The resulting latex can then be used, or the above-described DIR coupler is loaded into the cyan polymer coupler latex in a manner as described in Japanese Patent Application (OPI) Nos. 59942/76 and 32552/79, U.S. Pat. No. 4,199,363, etc., and the resulting latex can then be used.

Furthermore, the cyan polymer coupler latex according to the present invention can be used together with a DIR compound as described, for example, in West German Patent Application (OLS) Nos. 2,529,350, 2,448,063 and 2,610,546, U.S. Pat. Nos. 3,928,041, 3,958,993, 3,961,959, 4,049,455, 4,052,213, 3,379,529, 3,043,690, 3,364,022, 3,297,445 and 3,287,129.

Moreover, the cyan polymer coupler latex according to the present invention can be used in combination with a competing coupler as described, for example, in U.S. Pat. Nos. 3,876,428, 3,580,722, 2,998,314, 2,808,329, 2,742,832 and 2,689,793, etc., a stain preventing agent as described, for example, in U.S. Pat. Nos. 2,336,327, 2,728,659, 2,336,327, 2,403,721, 2,701,197 and 3,700,453, etc., a dye image stabilizing agent as described, for example, in British Pat. No. 1,326,889, U.S. Pat. Nos. 3,432,300, 3,698,909, 3,574,627, 3,573,050 and 3,764,337, etc., or the like.

The color photographic light-sensitive material produced according to the present invention can also contain conventionally well known coupler(s) other than a cyan color forming coupler. A non-diffusible coupler which contains a hydrophobic group, called a ballast group, in the molecule thereof is preferred as a coupler. A coupler can have either a 4-equivalent or a 2-equivalent property with respect to the silver ion. In addition, a colored coupler providing a color correction effect, or a coupler which releases a development inhibitor upon a development can also be present therein. Furthermore, a coupler which provides a colorless product upon coupling can be employed.

A known open chain ketomethylene type coupler can be used as a yellow color forming coupler. Of these couplers, benzoyl acetanilide type and pivaloyl acetanilide type compounds are especially effective. Specific examples of yellow color forming couplers which can be employed are described, for example, in U.S. Pat. Nos. 2,875,057, 3,265,506, 3,408,194, 3,551,155, 3,582,322, 3,725,072 and 3,891,445, West German Pat. No. 1,547,868, West German Patent Application (OLS) Nos. 2,219,917, 2,261,361 and 2,414,006, British Pat. No. 1,425,020, Japanese Patent Publication No. 10783/76, Japanese Patent Application (OPI) Nos. 26133/72, 73147/73, 102636/76, 6341/75, 123342/75, 130442/75, 21827/76 and 87650/75, etc.

A 5-pyrazolone coupler, a pyrazolobenzimidazole coupler, a cyanoacetyl cumaron coupler, an open chain acylacetonitrile coupler, etc. can be used as a magenta color forming coupler. Specific examples of magenta color forming couplers which can be employed are described, for example, in U.S. Pat. Nos. 2,600,788, 2,983,608, 3,062,653, 3,127,269, 3,311,476, 3,419,391, 3,519,429, 3,558,319, 3,582,322, 3,615,506, 3,834,908 and 3,891,445, West German Pat. No. 1,810,464, West Ger-

man Patent Application (OLS) Nos. 2,408,665, 2,417,945, 2,418,959 and 2,424,467, Japanese Patent Publication No. 6031/65, Japanese Patent Application (OPI) Nos. 20826/76, 58922/77, 129538/74, 74027/74, 159336/75, 42121/77, 74028/74, 60233/75, 26541/76 and 55122/78, etc.

Two or more kinds of the couplers described above can be incorporated into the same layer, or the same coupler compound can also be present in two or more layers.

A known method, for example, the method described in U.S. Pat. No. 2,322,027, can be used in order to incorporate the couplers described above into a silver halide emulsion layer. The coupler is dispersed in a hydrophilic colloid and then mixed with a silver halide emulsion. When a coupler having an acid group such as a carboxylic acid group, a sulfonic acid group, etc., is used, it can be incorporated into a hydrophilic colloid as an alkaline aqueous solution thereof.

The silver halide emulsions which can be used in the present invention are those wherein silver chloride, silver bromide, or a mixed silver halide such as silver chlorobromide, silver iodobromide, or silver chloroiodobromide is finely dispersed in a hydrophilic polymer such as gelatin. The silver halide can be chosen depending on the intended use of the photographic light-sensitive material from dispersions having a uniform grain size or those having a wide grain size distribution or from dispersions having an average grain size of from about 0.1 micron to 3 microns. These silver halide emulsions can be prepared, for example, by a single jet method, by a double jet method or a controlled double jet method, or by a ripening method such as an ammonia method, a neutral method, or an acid method. Also, these silver halide emulsions can be subjected to chemical sensitization such as a sulfur sensitization, a gold sensitization, a reduction sensitization, etc., and can contain a speed increasing agent such as a polyoxyethylene compound, an onium compound, etc. Further, a silver halide emulsion of the type wherein latent images are predominantly formed on the surface of the grains or of the type where latent images are predominantly formed inside the grains can be used in the present invention. Also, two or more kinds of silver halide photographic emulsions prepared separately and then mixed can be employed.

Suitable examples of a hydrophilic high molecular weight substance composed of the photographic light-sensitive layer of the present invention include a protein such as gelatin, etc., a high molecular weight non-electrolyte such as polyvinyl alcohol, polyvinyl pyrrolidone, polyacrylamide, etc., an acidic high molecular weight substance such as an alginate, a polyacrylic acid salt, etc., a high molecular weight amphotile such as a polyacrylamide treated with the Hoffman rearrangement reaction, a copolymer of acrylic acid and N-vinylimidazole, etc., a cross-linkable polymer such as those described in U.S. Pat. No. 4,215,195, and the like. Furthermore, a dispersion of a hydrophobic high molecular weight substance such as a latex of polybutyl acrylate, etc., can be included in the continuous phase of such a hydrophilic high molecular weight substance.

The silver halide emulsion used in the present invention can be chemically sensitized, as noted above, using conventional methods. Examples of suitable chemical sensitizers include, for example, a gold compound such as a chloroaurate and gold trichloride, as described in U.S. Pat. Nos. 2,399,083, 2,540,085, 2,597,856, and

2,597,915; a salt of a noble metal, such as platinum, palladium, iridium, rhodium and ruthenium, as described in U.S. Pat. Nos. 2,448,060, 2,540,086, 2,566,245, 2,566,263 and 2,598,079; a sulfur compound capable of forming silver sulfide by reacting with a silver salt, such as those described in U.S. Pat. Nos. 1,574,944, 2,410,689, 3,189,458 and 3,501,313; a stannous salt, an amine, and other reducing compounds such as those described in U.S. Pat. Nos. 2,487,850, 2,518,698, 2,521,925, 2,521,926, 2,694,637, 2,983,610 and 3,201,254 and the like.

Various compounds can be added to the photographic emulsions used in the present invention in order to prevent a reduction of the sensitivity or a formation of fog during preparation, storage, or processing. A wide variety of such compounds are known, such as a heterocyclic compound, mercury-containing compound, a mercapto compound or a metal salt, including 4-hydroxy-6-methyl-1,3,3a,7-tetraazaindene, 3-methylbenzothiazole and 1-phenyl-5-mercaptopurine, etc. Other examples of such compounds which can be used are described, for example, in U.S. Pat. Nos. 1,758,576, 2,110,178, 2,131,038, 2,173,628, 2,697,040, 2,304,962, 2,324,123, 2,349,198, 2,444,605-8, 2,566,245, 2,694,716, 2,697,099, 2,708,162, 2,728,663-5, 2,476,536, 2,824,001, 2,843,491, 2,886,437, 3,052,544, 3,137,577, 3,220,839, 3,226,231, 3,236,652, 3,251,691, 3,252,799, 3,287,135, 3,326,681, 3,420,668 and 3,622,339, British Pat. Nos. 893,428, 403,789, 1,173,609 and 1,200,188, as well as in K. Mees, *The Theory of the Photographic Process*, 3rd Ed. (1966) and the literature references cited therein.

The photographic emulsion used in the present invention can also contain a surface active agent individually or as a mixture thereof. These surface active agents are commonly used as a coating aid. However, in some cases they are used for the purposes of emulsion dispersion, sensitization, static prevention, adhesion prevention, etc.

The surface active agents can be classified into various groups, as follows: a natural surface active agent such as saponin, etc.; a nonionic surface active agent such as an alkylene oxide, a glycerol and a glycidol, etc.; a cationic surface active agent such as a high alkylamine, a quaternary ammonium salt, a heterocyclic compound such as pyridine and the like, a phosphoniums, a sulfoniums, etc.; an anionic surface active agent containing an acid group such as a carboxylic acid group, a sulfonic acid group, a phosphoric acid group, a sulfuric acid ester group, a phosphoric acid ester group, etc.; an amphoteric surface active agent such as an amino acid, an aminosulfonic acid, an aminoalcohol sulfuric acid ester, an aminoalcohol phosphoric acid ester, etc. Some examples of those surface active agents which can be used are described in U.S. Pat. Nos. 2,271,623, 2,240,472, 2,288,226, 2,739,891, 3,068,101, 3,158,484, 3,201,253, 3,210,191, 3,294,540, 3,415,649, 3,441,413, 3,442,654, 3,475,174, 3,545,974, West German Patent Application (OLS) No. 1,942,665, British Pat. Nos. 1,077,317 and 1,198,450, as well as Ryohi Oda et al., *Kainenkasseizai no Gosei to Sono Oyo (Synthesis and Application of Surface Active Agents)*, Maki Shoten (1964), A. W. Perry, *Surface Active Agents*, Interscience Publications, Inc. (1958) and J. P. Sisley, *Encyclopedia of Surface Active Agents*, Vol. II, Chemical Publishing Co. (1964), etc.

The photographic emulsion can be spectrally sensitized, or supersensitized, using a cyanine-type dye, such as a cyanine, merocyanine, carbocyanine, etc., individu-

ally, in combination, or in combination with a styryl dye.

These spectral sensitization techniques are well known, and are described, for example, in U.S. Pat. Nos. 2,688,545, 2,912,329, 3,397,060, 3,615,635 and 3,628,964, British Pat. Nos. 1,195,302, 1,242,588 and 1,293,862, West German Patent Application (OLS) Nos. 2,030,326 and 2,121,780, Japanese Patent Publication Nos. 4936/68 and 14030/69, etc. The sensitizers can be selected as desired depending on the wavelength range, sensitivity, etc. due to the purpose and use of the photographic light-sensitive material to be sensitized.

The hydrophilic colloid layer, and in particular a gelatin layer in the photographic light-sensitive material used in the present invention, can be hardened using various kinds of cross-linking agents. For instance, an inorganic compound such as a chromium salt, a zirconium salt, etc. or an aldehyde type cross-linking agent such as mucochloric acid, or 2-phenoxy-3-chloromalealdehydic acid as described in Japanese Patent Publication No. 1872/71 can be effectively used in the present invention. However, a non-aldehyde type cross-linking agent such as a compound having plural epoxy rings as described in Japanese Patent Publication No. 7133/59, a poly(1-aziridinyl) compound as described in Japanese Patent Publication No. 8790/62, an active halogen compound as described in U.S. Pat. Nos. 3,362,827 and 3,325,287, a vinyl sulfone compound as described in U.S. Pat. Nos. 2,994,611 and 3,582,322, Belgian Pat. No. 686,440, etc., are particularly suitable for use in the photographic light-sensitive material of the present invention.

The silver halide photographic emulsion according to the present invention is suitably applied to a support. Illustrative supports include a rigid material such as glass, a metal and a ceramic, and a flexible material and the type of support chosen depends on the end-use objects. Typical examples of flexible supports include a cellulose nitrate film, a cellulose acetate film, a polyvinyl acetal film, a polystyrene film, a polyethylene terephthalate film, a polycarbonate film and a laminate thereof, a baryta coated paper, a paper coated with an  $\alpha$ -olefin polymer, such as polyethylene, polypropylene and an ethylene-butene copolymer, a plastic film having a roughened surface as described in Japanese Patent Publication No. 19068/72, and the like. Depending upon the end-use objects of the photographic light-sensitive material, the support can be transparent, colored by adding a dye or pigment, opaque by adding, for example, titanium white, or light-shielding by adding, for example, carbon black.

The layer of the photographic light-sensitive material can be coated on a support using various coating methods, including a dip coating method, an air-knife coating method, a curtain coating method, an extrusion coating method using a hopper as described in U.S. Pat. No. 2,681,294. Also, two or more layers can be coated simultaneously, using methods as described in U.S. Pat. Nos. 2,761,791, 3,508,947, 2,941,898, 3,526,528, etc.

In order to incorporate a coupler into a silver halide emulsion layer, a known method, for example, the method as described in U.S. Pat. No. 2,322,027 can be employed. For example, the coupler may be dissolved in an organic solvent having a high boiling point, for example, a phthalic acid alkyl ester (e.g., dibutyl phthalate, diethyl phthalate, etc.), a phosphoric acid ester (e.g., diphenyl phosphate, triphenyl phosphate, tricresyl phosphate, diethylbutyl phosphate, etc.), a citric acid

ester (e.g., tributyl acetyl citrate, etc.), a benzoic acid ester (e.g., octyl benzoate, etc.), an alkyl amide (e.g., diethyl lauryl amide, etc.), a fatty acid ester (e.g., dibutoxyethyl succinate, dioctyl azelate, etc.), a trimersic acid ester (e.g., tributyl trimersate, etc.), etc., or in an organic solvent having a boiling point of from about 30° to about 150° C., for example, a lower alkyl acetate (e.g., ethyl acetate, butyl acetate, etc.), ethyl propionate, sec-butyl alcohol, methyl isobutyl ketone,  $\beta$ -ethoxyethyl acetate, methyl cellosolve acetate, etc., and then the solution is dispersed in a hydrophilic colloid. The above described organic solvent having a high boiling point and the above described organic solvent having a low boiling point may be used as mixture, if desired.

Furthermore, the dispersing method using a polymeric material as described in Japanese Patent Publication No. 39853/76 and Japanese Patent Application (OPI) No. 59943/76 can also be used.

When a coupler having an acid group, such as a carboxylic acid group, a sulfonic acid group, etc., is used, it can be incorporated in a hydrophilic colloid as an alkaline aqueous solution thereof.

The photographic light-sensitive material of the present invention may contain a ultraviolet light absorbing agent in a hydrophilic colloid layer. For example, a benzotriazole compound substituted with an aryl group, a 4-thiazolidone compound, a benzophenone compound, a cinnamic ester compound, a butadienen compound, a benzoxazole compound and an ultraviolet light absorbing polymer can be employed. These ultraviolet light absorbing agents may be fixed in the hydrophilic colloid layer.

Specific examples of the ultraviolet light absorbing agents are described, for example, in U.S. Pat. Nos. 3,533,794, 3,314,794 and 3,352,681, Japanese Patent Application (OPI) No. 2784/71, U.S. Pat. Nos. 3,705,805, 3,707,375, 4,045,229, 3,700,455 and 3,499,762, West German Patent Publication No. 1,547,963, etc.

In practice of the present invention, a known fade-preventing agent can be used. A color image stabilizing agent can be used alone individually or in combination two or more thereof. Examples of known fade-preventing agents include a hydroquinone derivative, a gallic acid derivative, a p-alkoxyphenol, a p-oxyphenol derivative or a biphenol, etc.

Specific examples of hydroquinone derivatives are described in U.S. Pat. Nos. 2,360,290, 2,418,613, 2,675,314, 2,701,197, 2,704,713, 2,728,659, 2,732,300, 2,735,765, 2,710,801 and 2,816,028, British Pat. No. 1,363,921, etc. Specific examples of gallic acid derivatives are described in U.S. Pat. Nos. 3,457,079 and 3,069,262, etc. Specific examples of p-alkoxyphenols are described in U.S. Pat. Nos. 2,735,765 and 3,698,909, Japanese Patent Publication Nos. 20977/74 and 6623/77, etc. Specific examples of p-oxyphenol derivatives are described in U.S. Pat. Nos. 3,432,300, 3,573,050, 3,574,627 and 3,764,337, Japanese Patent Application (OPI) Nos. 35633/77, 147434/77, and 15225/77, etc. Specific examples of bisphenols are described in U.S. Pat. No. 3,700,455.

The present invention is applicable to not only the so-called multilayer type photographic light-sensitive material comprising a support having superimposed thereon emulsion layers, each of which is sensitive to radiation of a substantially different wavelength region and forms color images of a substantially different hue, but also the so-called mixed packet type photographic

light-sensitive material comprising a support having coated thereon a layer containing packets which are sensitive to radiation of substantially different wavelength regions and form color images of a substantially different hue. The present invention can be applied to a color negative film, a color positive film, a color reversal film, a color printing paper, a color reversal printing paper, and the like.

The color photographic light-sensitive material of the present invention is, after exposure, subjected to a development processing to form dye images. Development processing includes basically a color development step, a bleaching step and a fixing step. Each step can be carried out individually or two or more steps can be combined as one step where a processing solution having two or more functions is used. Also, each step can be separated into two or more steps. The development processing can further include a pre-hardening step, a neutralization step, a first development (black-and-white development) step, a stabilizing step, a water washing step, and the like, if desired. The temperature of processing can be varied depending on the photographic light-sensitive material, the processing method, and the like. In general, the processing steps are carried out at a temperature from 18° C. to 60° C. These steps need not necessarily be conducted at the same temperature.

A color developer solution is an alkaline solution having a pH of more than 8, preferably from 9 to 12, and containing, as a developing agent, a compound whose oxidation product is capable of forming a colored compound when reacted with a color forming agent, i.e., a color coupler. The developing agent described above include a compound capable of developing an exposed silver halide and having a primary amino group on an aromatic ring, and a precursor which forms such compound. Typical examples of preferred developing agents are, for example, 4-amino-N,N-diethylaniline, 3-methyl-4-amino-N,N-diethylaniline, 4-amino-N-ethyl-N- $\beta$ -hydroxyethylaniline, 3-methyl-4-amino-N-ethyl-N- $\beta$ -hydroxyethylaniline, 4-amino-3-methyl-N-ethyl-N- $\beta$ -methanesulfonamidoethylaniline, 4-amino-N,N-dimethylaniline, 4-amino-3-methoxy-N,N-diethylaniline, 4-amino-3-methyl-N-ethyl-N- $\beta$ -ethoxyethylaniline, 4-amino-3-methoxy-N-ethyl-N- $\beta$ -methoxyethylaniline, 4-amino-3- $\beta$ -methanesulfonamidoethyl-N,N-diethylaniline, and a salt thereof (for example, a sulfate, a hydrochloride, a sulfite, a p-toluene sulfonate, and the like). Other developing agents such as those described in U.S. Pat. Nos. 2,193,015 and 2,592,364, Japanese Patent Application (OPI) No. 64933/73, L. F. A. Mason, *Photographic Processing Chemistry*, pages 226-229, Focal Press, London (1966), T. H. James, *The Theory of the Photographic Process*, 4th Edition, pages 315-320, Macmillan, New York (1977), etc., can be used. Further, an amino-phenol as described in T. H. James, *The Theory of the Photographic Process*, 4th Edition, pages 311-315, etc., can be used. Also, a 3-pyrazolidone developing agent can be used together with these developing agents.

The color developing solution can optionally contain various additives. Typical examples of such additives include an alkaline agent (for example, an alkali metal or ammonium hydroxide, carbonate or phosphate, etc.); a pH-adjusting agent or buffer (for example, a weak acid such as acetic acid, boric acid, etc., a weak base, or salt thereof, etc.); a developing accelerator (for example, various pyridinium compounds or cationic compounds

such as those described in U.S. Pat. Nos. 2,648,604 and 3,671,247; potassium nitrate; sodium nitrate; a condensation product of polyethylene glycol, and a derivative thereof such as those described in U.S. Pat. Nos. 2,533,990, 2,577,127 and 2,950,970; a nonionic compound such as a polythioether represented by those described in British Pat. Nos. 1,020,033 and 1,020,032; a polymeric compound having a sulfite ester group such as those described in U.S. Pat. No. 3,068,097; an organic amine such as pyridine and ethanolamine; benzyl alcohol; a hydrazine and the like); an anti-fogging agent (for example, an alkali metal bromide; an alkali metal iodide; a nitrobenzimidazole such as those described in U.S. Pat. Nos. 2,496,940 and 2,656,271; mercaptobenzimidazole; 5-methylbenztriazole; 1-phenyl-5-mercaptop-tetrazole; a compound for use in rapid processing such as those described in U.S. Pat. Nos. 3,113,864, 3,342,596, 3,295,976, 3,615,522 and 3,597,199; a thiosulfonyl compound such as those described in British Pat. No. 972,211; a phenazine-N-oxide such as those described in Japanese Patent Publication No. 41675/71; those described in *Kagaku Shashin Binran (Manual of Scientific Photography)*, Vol. II, pages 29-47, and the like); a strain or sludge preventing agent such as those described in U.S. Pat. Nos. 3,161,513 and 3,161,514, and British Pat. Nos. 1,030,442, 1,144,481 and 1,251,558; an interlayer-effect accelerator disclosed in U.S. Pat. No. 3,536,487; a preservative (for example, a sulfite, a bisulfite, hydroxyamine hydrochloride, formsulfite, a alkanolaminesulfite adduct, etc.) and the like.

The color photographic light-sensitive material of the present invention can be treated with various solutions prior to color development.

In the case of color reversal films, treatment with a first development solution is also carried out prior to the color development. As the first development solution, an alkaline aqueous solution containing at least one developing agent, such as hydroquinone, 1-phenyl-3-pyrazolidone, N-methyl-p-aminophenol and the like can be employed. The solution can also contain an inorganic salt such as sodium sulfate, etc.; a pH-adjusting agent or buffer such as borax, boric acid, sodium hydroxide and sodium carbonate, etc.; a development fog preventing agent such as an alkali metal halide (such as potassium bromide, etc.), and the like.

The additives illustrated above and the amounts thereof employed are well known in the color processing field.

After color development, the color photographic materials are usually bleached and fixed. The process can be effected in a blix bath which combines the bleaching and fixing steps. Various known compounds can be used as a bleaching agent, for example, a ferricyanide, a dichromate; a water-soluble iron (III) salt, a water-soluble cobalt (III) salt; a water-soluble copper (II) salt; a water-soluble quinone; a nitrosophenol, a complex salt of a polyvalent cation such as iron (III), cobalt (III), copper (II), etc., and an organic acid, for example, a metal complex of an aminopolycarboxylic acid such as ethylenediaminetetraacetic acid, nitrilotriacetic acid, iminodiacetic acid, N-hydroxyethylenediaminetriacetic acid, etc., malonic acid, tartaric acid, malic acid, diglycolic acid and dithioglycolic acid, and a copper complex salt of 2,6-dipicolinic acid; a peracid such as an alkylperacid, a persulfate, a permanganate and hydrogen peroxide; hypochlorite; chlorine; bromine; bleaching powder; and the like. These can be suitably used, individually or in combination. To the

bleaching solution, a bleaching accelerator such as those described in U.S. Pat. Nos. 3,042,520 and 3,241,966, Japanese Patent Publication Nos. 8506/70 and 9936/70 and various other additives can be added.

Any known fixing solution can be used for fixing the photographic material of the present invention. That is, ammonium, sodium, or potassium thiosulfate can be used as a fixing agent at a concentration of about 50 to about 200 g/liter. Fixing solution can further contain a stabilizer such as a sulfite and a metabisulfite; a hardener such as potassium alum; a pH buffer such as an acetate and a borate, and the like. The fixing solution generally has a pH of more than 3 or less.

Bleaching bath, fixing bath and blixing bath as described, for example, in U.S. Pat. No. 3,582,322, Japanese Patent Application (OPI) No. 101934/73, West German Pat. No. 1,051,117, etc. can also be employed.

The present invention will be explained in greater detail with reference to the following examples, but the present invention should not be construed as being limited thereto.

## EXAMPLE 1

On a paper support both surfaces of which were 25 laminated with polyethylene were coated a first layer (undermost layer) to a sixth layer (uppermost layer) as shown in Table below in order to prepare a color photographic light-sensitive material which is designated Sample 1. In Table below, a coating amount is set forth 30 in mg/m<sup>2</sup>.

|                                            |                                                                                                                                                                                                                                                                                                  |
|--------------------------------------------|--------------------------------------------------------------------------------------------------------------------------------------------------------------------------------------------------------------------------------------------------------------------------------------------------|
| Sixth Layer:<br>(Protective layer)         | Gelatin (1,000 mg/m <sup>2</sup> )                                                                                                                                                                                                                                                               |
| Fifth Layer:<br>(Red-sensitive<br>layer)   | Silver chlorobromide emulsion<br>(Silver bromide: 50 mol %;<br>silver: 300 mg/m <sup>2</sup> )<br>Cyan coupler* <sup>1</sup> (400 mg/m <sup>2</sup> ),<br>Coupler solvent* <sup>2</sup> (400 mg/m <sup>2</sup> ),<br>Gelatin (1,000 mg/m <sup>2</sup> )                                          |
| Fourth Layer:<br>(Intermediate layer)      | Ultraviolet light absorbing agent* <sup>3</sup><br>(1,000 mg/m <sup>2</sup> ),<br>Ultraviolet light absorbing agent<br>solvent* <sup>4</sup> (250 mg/m <sup>2</sup> ),<br>Gelatin (1,200 mg/m <sup>2</sup> )                                                                                     |
| Third Layer:<br>(Green-sensitive<br>layer) | Silver chlorobromide emulsion<br>(Silver bromide: 50 mol %;<br>silver: 290 mg/m <sup>2</sup> )<br>Magenta coupler* <sup>4</sup> (200 mg/m <sup>2</sup> ),<br>Coupler solvent* <sup>5</sup> (200 mg/m <sup>2</sup> ),<br>Gelatin (1,000 mg/m <sup>2</sup> )<br>Gelatin (1,000 mg/m <sup>2</sup> ) |
| Second Layer:<br>(Intermediate layer)      | Silver chlorobromide emulsion<br>(Silver bromide: 80 mol %;<br>silver: 400 mg/m <sup>2</sup> )<br>Yellow coupler* <sup>6</sup> (300 mg/m <sup>2</sup> )<br>Coupler solvent* <sup>7</sup> (150 mg/m <sup>2</sup> )<br>Gelatin (1,200 mg/m <sup>2</sup> )                                          |
| First Layer<br>(Blue-sensitive<br>layer)   | Paper support both surfaces of<br>which were laminated with poly-<br>ethylene                                                                                                                                                                                                                    |
| Support:                                   |                                                                                                                                                                                                                                                                                                  |

\*<sup>1</sup>Cyan coupler: 2-[ $\alpha$ -(2,4-Di-tert-pentylphenoxy)-butanamido]-4,6-dichloro-5-methoxyphenol

\*<sup>2</sup>Coupler solvent: Dibutyl phthalate

\*<sup>3</sup>Ultraviolet light absorbing agent: 2-(2-Hydroxy-3-sec-butyl-5-tert-butylphenyl)benzotriazole

\*<sup>4</sup>Magenta coupler: 1-(2,4,6-Trichlorophenyl)-3-(2-chloro-5-tetradecanamido)anilino-2-pyrazolin-5-one

\*<sup>5</sup>Coupler solvent: Tricresyl phosphate

\*<sup>6</sup>Yellow coupler:  $\alpha$ -Pivaloyl- $\alpha$ -(2,4-dioxo-5,5-dimethylazolidin-3-yl)-2-chloro-5-[ $\alpha$ -(2,4-di-tert-pentyl-

-continued

\*7Coupler solvent: phenoxy)butanamido]-acetanilide  
Diocetyl butyl phosphate

Sample 2 was prepared in the same manner as described in Sample 1 except that the cyan coupler solvent in Sample 1 was eliminated. Also, Sample 3 was prepared in the same manner as described in Sample 1 except that 400 mg/m<sup>2</sup> of oleophilic polymer coupler which was synthesized in the same manner as described in Synthesis Example 7 but using 6-methacrylamido-2,4-dichloro-3-methylphenol as a monomer coupler and methyl acrylate as a non-color forming monomer (containing 52.0% of the monomer coupler) was used in place of the cyan coupler in Sample 1 and that the cyan

-continued

|                                    |                    |
|------------------------------------|--------------------|
| Sodium Sulfite                     | 10 g               |
| Ammonium Thiosulfate (70% aq. sol) | 160 ml             |
| Sodium Ethylenediaminetetraacetate | 5 g                |
| Water to make                      | 100 ml<br>(pH 6.8) |

The spectral reflective density of each sample after development processing was measured using a spectral densitometer. The results thus obtained are shown in Table below. It is well known that hue of a cyan dye image is varied depending on a maximum absorption wavelength and a half width of absorption (particularly a shape of shorter wavelength side) which has influence on the color reproducibility.

| Sample | Maximum Absorption Wavelength | Wavelength at Position having Half Value of Maximum Absorption (shorter wavelength side) | Visual Evaluation          | Remarks           |
|--------|-------------------------------|------------------------------------------------------------------------------------------|----------------------------|-------------------|
| 1      | 650 nm                        | 563 nm                                                                                   | Preferable Blue            | Comparison        |
| 2      | 659 nm                        | 563 nm                                                                                   | Preferable Blue            | Comparison        |
| 3      | 660 nm                        | 568 nm                                                                                   | Sky Blue becomes yellowish | Comparison        |
| 4      | 660 nm                        | 564 nm                                                                                   | Preferable Blue            | Present Invention |
| 5      | 659 nm                        | 564 nm                                                                                   | Preferable Blue            | Present Invention |
| 6      | 659 nm                        | 562 nm                                                                                   | Preferable Blue            | Present Invention |
| 7      | 660 nm                        | 564 nm                                                                                   | Preferable Blue            | Present Invention |
| 8      | 659 nm                        | 564 nm                                                                                   | Preferable Blue            | Present Invention |

coupler solvent was eliminated. Further, Samples 4, 5, 6, 7 and 8 were prepared in the same manner as described in Sample 1 except that 500 mg/m<sup>2</sup> of Oleophilic Polymer Coupler (B), 500 mg/m<sup>2</sup> of Oleophilic Polymer Coupler (F), 600 mg/m<sup>2</sup> of Oleophilic Polymer Coupler (N), 500 mg/m<sup>2</sup> of Oleophilic Polymer Coupler (M) and 500 mg/m<sup>2</sup> of Polymer Coupler Latex (II) according to the present invention were used respectively in place of the cyan coupler in Sample 1 and that the cyan coupler solvent was eliminated.

Each sample was exposed to red light and subjected to development processing in the following manner.

| Processing Step    | Temperature | Time         |
|--------------------|-------------|--------------|
| Color Development  | 33° C.      | 3 min 30 sec |
| Bleach-Fixing      | 33° C.      | 1 min 30 sec |
| Washing with Water | 30° C.      | 3 min        |
| Drying             |             |              |

The processing solutions used in the color development processing had the following compositions:

| Color Development Solution                                       |                      |
|------------------------------------------------------------------|----------------------|
| Benzyl Alcohol                                                   | 15 ml                |
| Sodium Sulfite                                                   | 5 g                  |
| Potassium Bromide                                                | 0.4 g                |
| Hydroxylamine Sulfate                                            | 2 g                  |
| 4-(N-Ethyl-N-β-methanesulfonamido)-2-methylaniline sesquisulfate | 2 g                  |
| Sodium Carbonate (monohydrate)                                   | 30 g                 |
| Water to make                                                    | 1000 ml<br>(pH 10.1) |

  

| Bleach-Fixing Solution             |      |
|------------------------------------|------|
| Ferric Ethylenediaminetetraacetate | 45 g |

As is apparent from the results shown in Table above, the hue is varied depending on the wavelength of shorter wavelength side at the position having the half value of the maximum absorption rather than the maximum absorption wavelength. In Sample 3 wherein the polymer coupler which is out of the scope of the present invention was used the blue color of the sky was observed yellowish and thus desirable color reproduction can not be attained, only the wavelength of shorter wavelength side at the position having the half value of the maximum absorption was shifted 5 nm to the shorter wavelength side than that of Sample 1. On the contrary, the wavelength was hardly changed and the preferable hue was maintained in Samples 4 to 8 wherein the polymer couplers according to the present invention were used.

Further, the heat fastness of the cyan dye images obtained in the samples was measured. It was found that the cyan dye images obtained from the polymer couplers according to the present invention indicated the substantially same fastness to heat as those obtained from the polymer coupler for comparison.

## EXAMPLE 2

On a cellulose triacetate support were coated a first layer (undermost layer) to a sixth layer (uppermost layer) as shown in Table below in order to prepare a multilayer color photographic light-sensitive material which is designated Sample 9. In Table below, a coating amount is set forth in mg/m<sup>2</sup>.

|                                    |                                  |
|------------------------------------|----------------------------------|
| Sixth Layer:<br>(Protective layer) | Gelatin (750 mg/m <sup>2</sup> ) |
|------------------------------------|----------------------------------|

-continued

|                                         |                                                                                                                                                                                                                                                                                              |    |
|-----------------------------------------|----------------------------------------------------------------------------------------------------------------------------------------------------------------------------------------------------------------------------------------------------------------------------------------------|----|
| Fifth Layer;<br>(Green-sensitive layer) | Silver chlorobromide emulsion<br>(Silver bromide: 30 mol %;<br>silver: 500 mg/m <sup>2</sup> )<br>Magenta coupler* <sup>1</sup> (600 mg/m <sup>2</sup> )<br>Coupler solvent* <sup>2</sup> (110 mg/m <sup>2</sup> )<br>Gelatin (1,300 mg/m <sup>2</sup> )<br>Gelatin (500 mg/m <sup>2</sup> ) | 5  |
| Fourth Layer;<br>(Intermediate layer)   | Silver chlorobromide emulsion<br>(Silver bromide: 30 mol %;<br>silver: 500 mg/m <sup>2</sup> )<br>Cyan coupler* <sup>3</sup> (1,500 mg/m <sup>2</sup> )<br>Coupler solvent* <sup>4</sup> (700 mg/m <sup>2</sup> )<br>Gelatin (2,900 mg/m <sup>2</sup> )<br>Gelatin (500 mg/m <sup>2</sup> )  | 10 |
| Second Layer;<br>(Intermediate layer)   | Silver iodobromide emulsion<br>(Silver iodide: 0.2 mol %;<br>silver: 100 mg/m <sup>2</sup> )<br>Yellow coupler* <sup>5</sup> (1,200 mg/m <sup>2</sup> )<br>Coupler solvent* <sup>6</sup> (600 mg/m <sup>2</sup> )<br>Gelatin (2,200 mg/m <sup>2</sup> )<br>Gelatin (500 mg/m <sup>2</sup> )  | 15 |
| First Layer;<br>(Blue-sensitive layer)  | Silver iodobromide emulsion<br>(Silver iodide: 0.2 mol %;<br>silver: 100 mg/m <sup>2</sup> )<br>Yellow coupler* <sup>5</sup> (1,200 mg/m <sup>2</sup> )<br>Coupler solvent* <sup>6</sup> (600 mg/m <sup>2</sup> )<br>Gelatin (2,200 mg/m <sup>2</sup> )<br>Gelatin (500 mg/m <sup>2</sup> )  | 20 |
| Support                                 | Cellulose triacetate                                                                                                                                                                                                                                                                         |    |
| * <sup>1</sup> Magenta coupler:         | 3-[3-[2-(2,4-Di-tert-pentylphenoxy)-acetamido]benzamido]-1-(2,4,6-trichlorophenyl)-2-pyrazolin-5-one                                                                                                                                                                                         |    |
| * <sup>2</sup> Coupler solvent:         | Tricresyl phosphate                                                                                                                                                                                                                                                                          |    |
| * <sup>3</sup> Cyan coupler:            | 2-[ $\alpha$ -(2,4-Di-tert-pentylphenoxy)-butanamido]-4,6-dichloro-5-methylphenol                                                                                                                                                                                                            |    |
| * <sup>4</sup> Coupler solvent:         | Dibutyl phthalate                                                                                                                                                                                                                                                                            |    |
| * <sup>5</sup> Yellow coupler:          | $\alpha$ -Pivaloyl- $\alpha$ -(2,4-dioxo-5,5-dimethyloxazolidin-3-yl)-2-chloro-5-[ $\alpha$ -(2,4-di-tert-pentylphenoxy)-butanamido]acetanilide                                                                                                                                              |    |
| * <sup>6</sup> Coupler solvent:         | Tricresyl phosphate                                                                                                                                                                                                                                                                          |    |

Sample 10 was prepared in the same manner as described in Sample 9 except that the cyan coupler solvent in Sample 9 was eliminated. Also, Samples 11, 12, 13 and 14 were prepared in the same manner as described in Sample 9 except that 1,500 mg/m<sup>2</sup> of the polymer coupler used in Sample 3 in Example 1, and 1,900 mg/m<sup>2</sup> of Oleophilic Polymer Coupler (B), 1,800 mg/m<sup>2</sup> of Oleophilic Polymer Coupler (H) and 2,000 mg/m<sup>2</sup> of Oleophilic Polymer Coupler (T) according to the present invention were used respectively in place of the cyan coupler in Sample 9. Further, Samples 15, 16, 17 and 18 were prepared in the same manner as described in Samples 11, 12, 13 and 14 respectively except that the cyan coupler solvent was eliminated.

Each sample was exposed to blue light, green light and red light through a continuous wedge and subjected to the following development processing.

| Processing Step    | Temperature | Time   |
|--------------------|-------------|--------|
| Color Development  | 36° C.      | 3 min  |
| Stopping           | 36° C.      | 40 sec |
| First Fixing       | 36° C.      | 40 sec |
| Bleaching          | 36° C.      | 1 min  |
| Second Fixing      | 36° C.      | 40 sec |
| Washing with Water | 30° C.      | 30 sec |
| Drying             |             |        |

The processing solution used in the color development processing had the following compositions:

| Color Development Solution          |      |
|-------------------------------------|------|
| Sodium Sulfite                      | 5 g  |
| 4-Amino-3-methyl-N,N—diethylaniline | 3 g  |
| Sodium Carbonate                    | 20 g |

-continued

|                           |            |
|---------------------------|------------|
| Potassium Bromide         | 2 g        |
| Water to make             | 1 liter    |
|                           | (pH: 10.5) |
| <u>Stopping Solution</u>  |            |
| 6 N Sulfuric Acid         | 50 ml      |
| Water to make             | 1 liter    |
|                           | (pH: 1.0)  |
| <u>Fixing Solution</u>    |            |
| Ammonium Thiosulfate      | 60 g       |
| Sodium Sulfite            | 2 g        |
| Sodium Hydrogen Sulfite   | 10 g       |
| Water to make             | 1 liter    |
|                           | (pH: 5.8)  |
| <u>Bleaching Solution</u> |            |
| Potassium Ferricyanide    | 30 g       |
| Potassium Bromide         | 15 g       |
| Water to make             | 1 liter    |
|                           | (pH: 6.5)  |

20 The color density at the portion exposed to red light in each sample after development processing was measured. The fog, gamma and maximum density in each sample are shown in Table below.

| 25 | Sample | Fog  | Gamma | Maximum Density | Remarks           |
|----|--------|------|-------|-----------------|-------------------|
|    | 9      | 0.07 | 3.12  | 3.40            | Comparison        |
|    | 10     | 0.06 | 2.98  | 3.03            | Comparison        |
|    | 11     | 0.05 | 3.02  | 3.16            | Comparison        |
|    | 15     | 0.06 | 2.33  | 2.52            | Comparison        |
|    | 16     | 0.06 | 3.11  | 3.41            | Present Invention |
|    | 17     | 0.06 | 3.13  | 3.38            | Present Invention |
|    | 18     | 0.06 | 3.17  | 3.50            | Present Invention |
|    | 12     | 0.05 | 3.22  | 3.56            | Present Invention |
|    | 13     | 0.06 | 3.25  | 3.51            | Present Invention |
|    | 14     | 0.06 | 3.27  | 3.61            | Present Invention |

As is apparent from the results shown in Table above, in Samples 11 and 15 containing the polymer cyan coupler for comparison the color formation was inferior. On the contrary, Samples 12 to 14 and 16 to 18 containing the polymer cyan coupler according to the present invention had the excellent color forming property.

While the invention has been described in detail and with reference to specific embodiment thereof, it will be apparent to one skilled in the art that various changes and modifications can be made therein without departing from the spirit and scope thereof.

What is claimed is:

1. A silver halide color photographic light-sensitive material comprising a support having thereon a silver halide emulsion layer containing a cyan color image forming polymer coupler latex which is capable of forming a dye upon coupling with an oxidation product of an aromatic primary amine developing agent and which is a polymer or copolymer having a repeating unit derived from a monomer represented by the following general formula (I):



60 wherein  $\text{R}_1$  represents a hydrogen atom, a lower alkyl group containing from 1 to 4 carbon atoms or a chlorine atom;  $\text{R}_2$  represents a hydrogen atom or an unsubsti-

tuted or substituted alkyl group having from 1 to 4 carbon atoms; A<sub>1</sub> represents an unsubstituted or substituted alkylene group which may be a straight chain or a branched chain; A<sub>2</sub> represents an unsubstituted or substituted alkylene group which may be a straight chain or a branched chain, an unsubstituted or substituted aralkylene group or an unsubstituted or substituted phenylene group; B<sub>1</sub> represents —O—, —S—, —SO—, —SO<sub>2</sub>—, —CONH— or —COO—; B<sub>2</sub> represents —NHCO— or —OCO—; X represents a halogen atom; Y represents a hydrogen atom or a lower alkyl group having from 1 to 5 carbon atoms; Z represents a hydrogen atom, a halogen atom or a substituted alkoxy group; l represents 0 or 1; m represents 0 or 1; and n represents 0 or 1.

2. A silver halide color photographic light-sensitive material as claimed in claim 1, wherein the alkylene group represented by A<sub>1</sub> is an alkylene group having from 1 to 10 carbon atoms.

3. A silver halide color photographic light-sensitive material as claimed in claim 1, wherein the alkylene group represented by A<sub>2</sub> is an alkylene group having from 1 to 10 carbon atoms.

4. A silver halide color photographic light-sensitive material as claimed in claim 1, wherein the substituent for the substituted alkylene group, the substituted aralkylene group or the substituted phenylene group represented by A<sub>1</sub> or A<sub>2</sub> is an aryl group, a nitro group, a hydroxy group, a cyano group, a sulfo group, an alkoxy group, an aryloxy group, an acyloxy group, an acylamino group, a sulfonamido group, a sulfamoyl group, a halogen atom, a carboxy group, a carbamoyl group, an alkoxy carbonyl group or a sulfonyl group.

5. A silver halide color photographic light-sensitive material as claimed in claim 1, wherein the substituent for the substituted alkoxy group represented Z is an aryl group, a nitro group, a hydroxy group, a cyano group, a sulfo group, an alkoxy group, an aryloxy group, an acyloxy group, an acylamino group, an alkylsulfonamido group, an alkylsulfamoyl group, a halogen atom, a carboxy group, an alkylcarbamoyl group, an alkoxy carbonyl group, an alkylsulfonyl group or an alkylthio group.

6. A silver halide color photographic light-sensitive material as claimed in claim 1, wherein the cyan color image forming polymer coupler latex comprises a polymer or copolymer having a repeating unit derived from a monomer represented by the following general formula (I'):



wherein R<sub>1</sub>, R<sub>2</sub>, A<sub>1</sub>, X, Y and Z each has the same meaning as defined in claim 1.

7. A silver halide color photographic light-sensitive material as claimed in claim 1, wherein the polymer is a homopolymer.

8. A silver halide color photographic light-sensitive material as claimed in claim 1, wherein the polymer is a copolymer.

9. A silver halide color photographic light-sensitive material as claimed in claim 8, wherein the copolymer contains a repeating unit derived from a non-color

forming monomer which does not couple with the oxidation product of an aromatic primary amine developing agent.

10. A silver halide color photographic light-sensitive material as claimed in claim 9, wherein the non-color forming monomer is an ester of acrylic acid, an amide of acrylic acid, a vinyl ester, an acrylonitrile, an aromatic vinyl compound, itaconic acid, citraconic acid, crotonic acid, vinylidene chloride, a vinyl alkyl ether, an ester of maleic acid, N-vinyl-2-pyrrolidone, N-vinyl pyridine, or 2- or 4-vinyl pyridine.

11. A silver halide color photographic light-sensitive material as claimed in claim 9, wherein the non-color forming monomer is an acrylic acid ester, a methacrylic acid ester or a maleic acid ester.

12. A silver halide color photographic light-sensitive material as claimed in claim 1, wherein the amount of the color forming portion in the polymer latex is from 5% to 80% by weight.

13. A silver halide color photographic light-sensitive material as claimed in claim 1, wherein the amount of the color forming portion in the polymer latex is from 20% to 70% by weight.

14. A silver halide color photographic light-sensitive material as claimed in claim 12, wherein the gram number of the polymer latex containing 1 mol of coupler monomer is from 250 to 4,000.

15. A silver halide color photographic light-sensitive material as claimed in claim 1, wherein the cyan color image forming polymer coupler latex is a latex prepared by emulsion polymerization of a monomer comprising a monomer coupler represented by the general formula (I).

16. A silver halide color photographic light-sensitive material as claimed in claim 1, wherein the cyan color image forming polymer coupler latex is a latex prepared by dissolving an oleophilic polymer coupler obtained by polymerization of a monomer comprising a monomer coupler represented by the general formula (I) in an organic solvent and then dispersing the solution in a latex form in an aqueous gelatin solution.

17. A silver halide color photographic light-sensitive material as claimed in claim 1, wherein the silver halide emulsion layer containing a cyan color image forming polymer coupler latex is a red-sensitive silver halide emulsion layer.

18. A silver halide color photographic light-sensitive material as claimed in claim 17, wherein the photographic light-sensitive material further comprises a blue-sensitive silver halide emulsion layer containing a yellow color image forming coupler and a green-sensitive silver halide emulsion layer containing a magenta color image forming coupler.

19. A method of forming a color image comprising developing an imagewise exposed silver halide color photographic light-sensitive material comprising a support having thereon a silver halide emulsion layer containing a cyan color image forming polymer coupler latex which is capable of forming a dye upon coupling with an oxidation product of an aromatic primary amine developing agent and which is a polymer or copolymer having a repeating unit derived from a monomer represented by the following general formula (I):



wherein R<sub>1</sub> represents a hydrogen atom, a lower alkyl group containing from 1 to 4 carbon atoms or a chlorine atom; R<sub>2</sub> represents a hydrogen atom or an unsubstituted or substituted alkyl group having from 1 to 4 carbon atoms; A<sub>1</sub> represents an unsubstituted or substituted alkylene group which may be a straight chain or

10  
15

a branched chain; A<sub>2</sub> represents an unsubstituted or substituted alkylene group which may be a straight chain or a branched chain, an unsubstituted or substituted aralkylene group or an unsubstituted or substituted phenylene group; B<sub>1</sub> represents —O—, —S—, —SO—, —SO<sub>2</sub>—, —CONH— or —COO—; B<sub>2</sub> represents —NHCO— or —OCO—; X represents a halogen atom; Y represents a hydrogen atom or a lower alkyl group having from 1 to 5 carbon atoms; Z represents a hydrogen atom, a halogen atom or a substituted alkoxy group; l represents 0 or 1; m represents 0 or 1; and n represents 0 or 1.

\* \* \* \* \*

20

25

30

35

40

45

50

55

60

65